

Patented Nov. 11, 1924.

1,515,504

# UNITED STATES PATENT OFFICE.

JAMES HENRY McDANIEL, OF WASHINGTON COURT HOUSE, OHIO.

## METHOD OF TREATING WOOD.

No Drawing.

Application filed April 7, 1924. Serial No. 704,881.

To all whom it may concern:

Be it known that I, JAMES HENRY McDANIEL, a citizen of the United States, and a resident of Washington Court House, in the county of Fayette and State of Ohio, have invented certain new and useful Improvements in Methods of Treating Wood, of which the following is a specification.

This invention relates to a method for the treatment of wood and has for its object the provision of a process for neutralizing wood separators which are employed for insulating storage batteries and in which the wood is impregnated with a water soluble chemical which will neutralize the natural acid content and render the natural vegetable oils chemically inactive.

This invention will be best understood from a consideration of the following detailed description; nevertheless it is to be understood that the invention is not confined to the disclosure, being susceptible of such changes and modifications which shall define no material departure from the salient features of the invention as expressed in the appended claims.

In carrying out my invention the wood cut to the shape of the insulators must be treated with a water soluble chemical such as an aqueous solution of sodium bisulphide dissolved in clear water, in the proportion by weight of 1 to 3, an alkali solution of caustic soda consisting of 10% by weight of the soda and 90% by weight of water, or an aqueous salt solution of potassium permanganate, containing 10% of the potassium salt and 90% water.

These solutions when combined or used separately and impregnated in the wood will neutralize the natural acid content and the natural vegetable oils so that the wood will be free of such elements which are deleterious to the flow of current and the electrolysis of the metal plates of a battery that are insulated by the wood, and furthermore by such treatment the cells of the wood will not break down by long immersion.

The wood shaped to size are placed in a retort which is hermetically sealed and a vacuum drawn. The water soluble chemical is introduced into the retort from a charging tank in a manner that the degree of vacuum is not disturbed and the vacuum is maintained for a period which will insure a rapid impregnation of the wood with the chemical solution.

When the retort or treating cylinder is filled with the solution, a hydrostatic pressure is then produced by pumping the neutralizing solution into the retort from charging tanks until a pressure is obtained that will insure a sufficient penetration of the wood by the neutralizing solution. The solution is heated by means of steam coils in the charging tank to a temperature of 100 degrees F. or to a predetermined temperature to insure penetration but which will not be injurious to the wood cells. A temperature is maintained in the retort by the steam coils in advance of the admission of the solution to maintain the temperature of the solution when introduced into the retort from the charging tanks.

At the end of the impregnating period the solution is then forced back to the charging tanks by means of pumps or air pressure. After draining the retort of solution a vacuum is drawn in the retort of sufficient degree and duration to recover that portion of the free solution in the wood that can be drawn out, which is then drained off.

The wood is then subjected to a similar process in which clear water is used as a leach, at a temperature not exceeding 100 degrees F. with a subsequent final vacuum drawn of sufficient degree and duration to recover as much of the water from the wood as has been predetermined so the wood will retain a certain amount of moisture not deleterious to its use.

What I claim is:

1. A process for forming wood separators for batteries which comprises placing wood cut to shape in a retort, creating a vacuum in the tank, charging a solution of sodium bisulphide, sodium hydroxide, and potassium permanganate into the retort, maintaining the solution under pressure and heating the same to 100 degrees F., withdrawing the solution, again creating a vacuum in the retort, charging fresh water into the retort, and maintaining the same under pressure and heating the water to approximately 100 degrees F., removing the water and again creating a vacuum in the retort.

2. A process for forming wood separators for batteries which comprises placing wood cut to shape in a retort, charging a solution of sodium bisulphide, sodium hydroxide, and potassium permanganate into the retort, maintaining the solution under pres-

sure and heating the same to 100 degrees F., withdrawing the solution, creating a vacuum in the retort, charging fresh water into the retort, and maintaining the same under pressure and heating the water to approximately 100 degrees F., removing the water and again creating a vacuum in the retort.

3. A process for forming wood separators for batteries which comprises placing wood cut to shape in a retort, creating a vacuum in the tank, charging a solution of sodium bisulphide, sodium hydroxide and potassium permanganate into the retort, heating said solution approximately 100 degrees F., withdrawing the solution and then charging fresh water into the retort, maintaining the same under pressure and heating the water to approximately 100 degrees F., removing the water and again creating a vacuum in the retort.

4. A process for forming wood separators for batteries which comprises placing wood cut to shape in a retort, charging a solution of sodium bisulphide, sodium hydroxide, and potassium permanganate into the retort, maintaining the solution under pres-

sure and heating the same to 100 degrees F., withdrawing the solution, and creating a vacuum in the retort.

5. A process for forming wood separators for batteries which comprises placing wood cut to shape in a retort, creating a vacuum in the tank, charging a solution of sodium bisulphide, sodium hydroxide, and potassium permanganate into the retort, maintaining the solution under pressure and heating the same to 100 degrees F., withdrawing the solution, and creating a vacuum in the retort.

6. A solution for neutralizing acids and vegetable oils in wood comprising an aqueous solution of sodium bisulphide in the proportions of 25% by weight and 75% by weight of water, an aqueous solution of sodium hydroxide consisting of 10% by weight of sodium hydroxide and 90% by weight of water, and an aqueous salt solution of potassium permanganate, containing 10% by weight of potassium permanganate and 90% by weight of water.

JAMES HENRY McDANIEL.